

## UNITED STATES PATENT OFFICE

JAMES H. CARMICHAEL, OF LOWELL, MASSACHUSETTS, ASSIGNOR, BY MESNE ASSIGNMENTS, TO WINCHESTER REPEATING ARMS COMPANY, A CORPORATION OF DELAWARE

## COATING SHOT SHELLS

• No Drawing.

Application filed December 15, 1928. Serial No. 326,418.

This invention relates to the manufacture of shot shells.

The typical shot shell consists of a metal case adapted to receive a primer and a charge of propellant powder. A cylindrical paper shell is arranged in the metal case and holds the charge and a paper or cardboard disc in the form of a wad is arranged in the upper end of this cylinder to retain the charge 10 therein. The end of the paper cylinder is crimped over the outer face of the wad to prevent its displacement. The paper or cardboard used in forming the wad and cylinder is preferably coated or impregnated with 15 paraffin.

It has been proposed to coat the exterior of shot shells with lacquer, varnish or other waterproof coatings and particularly to coat them with a lacquer having a nitrocellulose 20 base.

In coating the shot shells they are generally dipped into a tank containing the varnish, lacquer or other waterproof coating and a film or coating of the lacquer or varnish 25 placed over the entire shell. In practicing this process, several difficulties have been encountered. If the shot shells are cold when they are dipped, bubbles are apt to form on the top wad in the angle between it and the 30 crimp at the top of the paper cylinder and it is also difficult to obtain a smooth, uniform coating. I have found that these difficulties can be avoided by heating the shells before 35 they are dipped into the varnish or lacquer. The heating of the shells not only avoids the formation of bubbles on the top wad but also produces a smoother, more uniform coating that materially enhances the appearance of 40 the shot shell.

In practicing my improved process, the shells are first heated and then dipped into the lacquer, varnish or other waterproof coating in the same manner as heretofore. Care must be taken to prevent heating of 45 the shot shells to a temperature that would cause the paraffin on the paper cylinder and wad to melt. I accordingly preferably heat the shells to a temperature of about 110° F. or at any rate to a temperature substantially 50 below the melting point of the paraffin. The

heated shells are then dipped into the lacquer, varnish or other waterproof coating and when removed after the dipping operation and dried a superior product is obtained. As stated above, the bubbles which 55 have heretofore formed on the top wad in the angle between it and the crimp are avoided and a smoother, more uniform coating is obtained.

In some instances I have found it advisable to heat the shells a second time as they come out of the lacquer, but this second heating is not essential in most cases and the invention is not limited thereto.

## I claim:

1. The process of coating loaded shot shells consisting essentially of heating the shell to be coated and then coating it with a waterproof coating composition.

2. The process of coating loaded shot shells consisting essentially of heating a shell to a temperature of substantially 110° F. and then dipping the heated shell into a waterproof lacquer.

3. The process of coating loaded shot shells consisting essentially of heating the shell, dipping it into a waterproof lacquer while in heated condition and then heating the coated shell.

In testimony whereof I affix my signature.

JAMES H. CARMICHAEL.

65

70

75

85

90

95

100